

# UNITED STATES PATENT OFFICE.

GARLAND N. WHISTLER, OF FORT WADSWORTH, AND HENRY C. ASPINWALL, OF WEST NEW BRIGHTON, ASSIGNEES, BY MESNE ASSIGNMENTS, TO BENJAMIN S. HARMON, OF NEW YORK, N. Y.

## SMOKELESS GUNPOWDER.

SPECIFICATION forming part of Letters Patent No. 541,910, dated July 2, 1895.

Application filed October 23, 1894. Serial No. 528,735. (No specimens.)

*To all whom it may concern:*

Be it known that we, GARLAND N. WHISTLER, of Fort Wadsworth, and HENRY C. ASPINWALL, of West New Brighton, in the county of Richmond and State of New York, have invented a new and useful Improvement in Smokeless Gunpowder, of which the following is a specification.

Our invention relates to an improvement in smokeless gun powder in which the relative proportions of gun cotton and nitroglycerin may be varied within broad limits, at will, without materially affecting the propelling efficiency of the powder.

Smokeless powder, considered in its broad sense as an explosive, may be used either as a mining powder or as a gun powder. Its value as a mining powder depends simply upon the amount of gas developed and the temperature of explosion and is entirely independent of the rate of combustion. When used as a gun powder or propellant to propel a projectile through the bore of a gun, the object is to obtain the greatest velocity with the least strain upon the gun. The character of the pressure produced in the bore of a gun is dependent upon the rate of combustion of the powder. The propellant efficiency of a powder is therefore a result not only of the force of the powder but also of the rate of combustion.

The rate of combustion of nitroglycerin, so long as it does not detonate is peculiarly suitable for propelling purposes, whereas the rate of burning of gun cotton is too rapid and produces too great pressure. A mixture of these two explosives in certain proportions produces a safe compound which will not detonate and is a good propellant. The greater the amount of nitroglycerin, the more suitable will be the rate of combustion. In order, however, to obtain the most efficient propellant that the compound will produce, it is necessary to use an excessive amount of nitroglycerin; which is not only dangerous, but in consequence of nitroglycerin being a liquid, the grain produced by the combination is too soft for practical use in the gun. The decrease of the relative proportion of nitroglycerin, as compared with the gun cotton hardens the grain and renders it better suited

for the purpose of a gun powder, but at the same time decreases the efficiency of the gun powder as a propellant.

Our invention consists in combining with the gun cotton and the nitroglycerin from forty per cent. to fifty per cent. of the weight of gun cotton of some nitrate, such for example as barium nitrate, thereby rendering the rate of combustion of the gun cotton similar to that of the nitroglycerin and hence rendering it feasible to vary the relative proportions of gun cotton and nitroglycerin at will, without materially affecting the propellant efficiency of the powder. The gun cotton referred to is in the form known as "trinitrocellulose."

We have demonstrated in practice that a powder composed of one hundred and fifty parts of nitroglycerin; fifty parts trinitrocellulose, twenty-two and one-half parts of barium nitrate and two and one-half parts of urea crystals, gives the projectile in the United States thirty caliber rifle a velocity of about two thousand two hundred and fifty feet per second with a maximum pressure of thirty-eight thousand pounds per square inch. A second powder consisting of seventy-five parts of nitroglycerin, fifty parts of trinitrocellulose, twenty parts of barium nitrate and two parts of urea crystals give, in the same gun, with the same pressure, about two thousand two hundred and sixty feet per second.

It will be noticed, that the amount of barium nitrate was in the first instance about forty-five per cent. of the trinitrocellulose and in the latter case about forty per cent. of the gun cotton, and it is probable that further experience will show that the percentage of the barium nitrate may be varied slightly between these two per cents. as the proportion of nitroglycerin is decreased. It is of the highest importance, however, to observe that in the second instance the amount of nitroglycerin was only half as much again as the amount of trinitrocellulose, while, in the first instance, it was three times as much, and yet the propellant efficiency was about the same in both cases, varying only a few feet. We have shown therefore that, by the addition of a proportion of a salt, rich in oxygen, to the trinitrocellulose and nitroglycerin,

we can vary the proportions of the two explosives, nitroglycerin and trinitrocellulose, at will, without affecting the propellant efficiency of the powder, thus admitting of regulating the hardness of the grain to any extent that may be desirable and reducing the nitroglycerin to a safer proportion.

Instead of using barium nitrate, we may use potassium nitrate, calcium nitrate, strontium nitrate, ammonium nitrate or any other nitrate.

What we claim is—

A smokeless powder, composed of nitroglyc-

erine, trinitrocellulose, a nitrate and a neutralizer of free acid, such for example as urea 15 crystals, the proportion of nitrate to the trinitrocellulose being about forty-five parts of nitrate to one hundred parts of trinitrocellulose, so that the combustion of the gun cotton shall be substantially similar to that of the nitro-glycerin, as set forth.

GARLAND N. WHISTLER.  
HENRY C. ASPINWALL.

Witnesses:

IRENE B. DECKER,  
FREDK. HAYNES.